

Sept. 5, 1933.

1,925,391

E. J. KOHLMAYER  
PROCESS FOR THE RECOVERY OF IRON FROM IRON AND SULPHUR  
CARRYING METALLURGICAL PRODUCTS, ESPECIALLY ORES  
Filed Aug. 31, 1931

*Fig. 1*



*Fig. 2*



Ernst Justus Kohlmeier

INVENTOR

BY

Mack & Blum

ATTORNEYS

## UNITED STATES PATENT OFFICE

1,925,391

PROCESS FOR THE RECOVERY OF IRON  
FROM IRON AND SULPHUR CARRYING  
METALLURGICAL PRODUCTS, ESPECIALLY  
ORES

Ernst Justus Kohlmeyer, Berlin, Germany

Application August 31, 1931, Serial No. 560,509,  
and in Germany February 23, 1931

5 Claims. (Cl. 75—60)

The present invention is based on efforts to discover a simple smelting process for iron ores and other metallurgical products containing impurities, such as sulphur, to a high degree. Particular attention was directed to the discovery of a simple process for smelting pyrites with zinc-blende contents and also for zinc carrying roasted pyrites. It is naturally practicable to equally use the process for smelting pyrites free from zinc or pyrites containing or not impurities of another nature and also sulphur carrying roasted pyrites of any sort.

The principle of the invention is twofold: (1.) If it refers to oxydic products of iron with not too high sulphur content, this is used to convert the iron oxide into an iron-iron sulphide alloy with a relatively low sulphur content by means of a smelting process. (2.) If on the other hand it is a question of smelting products with a high sulphur content, as f. i. pyrites, the final aim is to produce a similar iron-iron sulphide alloy by partial oxidation or a dissociation plus oxidation of the sulphide-sulphur respectively.

As a final result of smelting each of these classes of ores, both of the sulphidic pyrites and the oxidic roasted pyrites, for which a special smelting process is described later, a gangue-free alloy merely containing Fe—FeS is to be produced in every case, which may be converted into iron directly or indirectly.

Smelting tests, the results of which are later given in detail, led to the realization of the principle that in all cases it is possible to obtain in a single operation a product, consisting of iron with 8-12% sulphur or of about 65-78% iron (Fe) and 22-35% of ferrous sulphide (FeS). It made little difference, although the steps varied somewhat in the details, whether the process was started with more oxidic or more sulphidic materials. It is evident that a greatly simplified iron production process can be based on such a fairly precisely definable product, which at the same time is free from gangue or other metallic impurities, than with any intermediate products and ores containing the most varied sorts of gangue or other admixtures.

The possibilities of converting this product into metallic iron will be referred to at the end of the description.

It seems advisable to first describe the necessary details regarding the observations during the tests, which led to obtaining this product and also some information regarding the properties of this iron-iron sulphide alloy and it seems con-

ducive to a better understanding to first say something with regard to the properties or action respectively of the several substances used in the process.

The materials which are treated are ferric-oxide, ferrous oxide, pyrite and ferrous sulphide and coal as solid or molten substances, whilst as gases air sulphur-dioxide and carbon monoxide are to be dealt with:

$\text{Fe}_2\text{O}_3$ — $\text{FeO}$ —C— $\text{FeS}_2$ — $\text{FeS}$ — $\text{SO}_2$ —CO—air. 65

The problem to be solved by applicant was to obtain a chemical equilibrium of these substances, so that only a phase of complete fusion of  $\text{Fe}$ — $\text{FeS}$  with  $\text{Fe}$  in excess is formed; since known 70 and reliable figures and facts about this equilibrium were so far not available, smelting tests had to be made.

In this respect only the properties of the individual substances were known till now. 75

Pyrite ( $\text{FeS}_2$ ) dissociates from about 550° C. and possesses at somewhat over 700° C. a sulphur vapor pressure of 1 atm. all temperatures, which are stated in this specification being given in the C. scale. On heating pyrite in a non-oxidizing 80 atmosphere it is converted into iron-monosulphide ( $\text{FeS}$ ) with a little metallic Fe, which has a melting point of about 1195° C.

On heating pyrite in air, i. e. an oxidizing atmosphere the same will, according to the size of 85 the grain, start to turn into iron oxide and sulphur dioxide at temperatures between 325 and 470° C.

Ferric-oxide ( $\text{Fe}_2\text{O}_3$ ) has a melting point of about 1565°, when the same dissociates partly into 90  $\text{Fe}_3\text{O}_4$  with a solidification point of about 1527°. This dissociation of the  $\text{Fe}_2\text{O}_3$  already commences in the atmospheric air at about 1370°, without however leading to the formation of  $\text{FeO}$ .  $\text{FeO}$  can only be produced by the reduction of iron oxide by coal or carbon monoxide. Without these reducing substances being present it is technically most difficult to keep it in a free form in the absence of silica, so that the alleged melting point of about 1360° is only of scientific interest 100 and is besides not to be relied upon. Smelting baths of pure ferrous oxide will therefore hardly be produced industrially in metallurgical practice by the means employed so far, as they would oxidize into magnetite at the normal furnace atmosphere, be it by the air or by carbon dioxide; nor could a complete fusion of molten ferric oxide ( $\text{Fe}_2\text{O}_3$ ) be produced as it would dissociate into magnetite ( $\text{Fe}_3\text{O}_4$ ).

Now as regards sulphidic molten baths of iron 110

such as  $\text{FeS}_2$ , as can be seen from the above explanations, they cannot exist without the use of extreme pressure, since they dissociate into  $\text{FeS}$ , which at the usual temperature of the metallurgical furnaces of between 1200 to 1500° in a non-oxidizing atmosphere cannot be further dissociated than what would correspond to a sulphur content of 28-32%. This sulphur content corresponds to a composition of 80-85%  $\text{FeS}$  and 20-15% Fe. The eutectic i. e. the lowest melting point of fused solutions of Fe with  $\text{FeS}$  lies at 84%  $\text{FeS}$  16% Fe and at a temperature of 985°. Practical experience has shown that in the usual smelting of pyrites or iron sulphides de-sulphurization by dissociation does not permit to exceed the eutectic point to any noticeable degree. Just as oxidic iron has its most stable form when fused as  $\text{Fe}_3\text{O}_4$  (thus neither  $\text{FeO}$  nor  $\text{Fe}_2\text{O}_3$ ) also the iron sulphur compound denotes its most stable form in a fused state and in a non-oxidizing furnace atmosphere at the aforementioned eutectic composition.

Except such cases in which  $\text{FeS}$  or its eutectic iron alloy together with lead sulphide or sulphide of copper occurs in the well known form of copper matte, this fused iron sulphide has so far hardly played a role worth mentioning, more especially in the direct recovery of iron. This is easily understood, since a sulphidic iron product with a 30% sulphur content did not offer any essential different workability than that of pyrites with a higher sulphur content.

In view of the great affinity of iron for oxygen if such a melt is treated with air as usual, the iron will be oxidized at the same time as the sulphur. It is known that in bessemerizing copper-matte, consisting of molten iron sulphide and copper sulphide, all iron is oxidized besides the sulphur.

It would thus be obviously of advantage, were it possible, to only oxidize the sulphur in a melt corresponding for instance to the eutectic composition above referred to, i. e. to enrich the melt with metallic iron to such an extent,—without at the same time oxidizing any appreciable quantity of iron—up to a point where a rapid working up of the molten product now containing a large percentage of iron against little iron sulphide, were possible. For it had been ascertained by tests that amongst the number of iron-iron sulphide alloys, which on the iron sulphide side had shown the eutectic point of 985°, there was on the iron side a technically remarkable point, which may be taken with about 8% of sulphur to correspond to about 75% Fe—25%  $\text{FeS}$ . In the diagram of the  $\text{Fe}$ — $\text{FeS}$  alloys the remarkable significance of this composition finds no expression since no new structural components are in any way perceptible from this point on. At the most it was possible to ascertain, that starting from this point the temperatures of solidification from the point of the primary solidification, which had risen but slowly with a decreasing sulphur content, were now rising rapidly. This turning point in primary solidification lies with pure materials at about 1375°.

The technically remarkable discovery now consists in that chilled products, which lie from this point towards the pure  $\text{FeS}$ , show a pronounced non-metallic character and can therefore be easily broken up in desintegrating apparatus. Those products, however, which lie from this point toward iron assume rapidly an increasing metallic character and therefore cannot be or can only with difficulty be disintegrated.

Since it has been found that by appropriate

treatment of a melt rich in sulphur by oxidation with air under a layer of coal the same can be freed from sulphur up to 8% without perceptibly oxidizing the iron this offers the means of obtaining a product which can be converted in a sintering plant into iron oxide agglomerate in one operation. The opportunity of making use of this chance is offered when dealing with pyrites with which other sulphides of a vaporizable nature are combined in a complex form as f. i.  $\text{ZnS}$ ,  $\text{PbS}$ ,  $\text{Bi}_2\text{S}_3$ ,  $\text{As}_2\text{S}_3$  etc.

Pure pyrites i. e., pyrites without such impurities would not be subjected to such a treatment, because they can be converted by a roasting and sintering process without fusion into iron oxide sinter. But since it is known by experience, that complex volatile metallic sulphides of the above kind can hardly be removed from the charge by the usual sintering processes, a conversion of such complex pyrites into a molten condition is essential for their direct removal from the charge. The present process makes it possible to deprive this iron sulphide melt of its sulphur to such an extent that an  $\text{Fe}$ — $\text{FeS}$ —melt of a low sulphur content is formed which can without any difficulty be worked up by granulation with a succeeding treatment in sintering apparatus into pure iron oxide sinter.

It has been stated that the process is particularly suited for pyrites containing other volatile metallic sulphides. This remark however also applies to pyrites containing appreciable quantities of gangue f. i. silica. If such pyrites are directly converted into ferric oxide sinter by sintering plants, the  $\text{Fe}_2\text{O}_3$  content of the sinter is seriously affected by the remaining gangue. If therefore such raw materials containing gangue and particularly  $\text{SiO}_2$  are subjected to the fusion process of this application, which has to be carried out in an atmosphere appropriate for reduction, so that if possible no  $\text{FeO}$ ,  $\text{Fe}_3\text{O}_4$  or  $\text{Fe}_2\text{O}_3$  is formed, the largest part of the sulphidic iron may be separated from the gangue, whereupon this sulphidic iron, on being subjected to the above mentioned treatment will yield a ferric-oxide sinter free from gangue and therefore of a high value.

Just to give an example:

There are such roasted products which have been obtained by ordinary roasting of zinc carrying pyrites. Such products contain zinc to the extent of a few percents as oxide otherwise in sulphidic form, therefore also a few percent of sulphur, besides gangue and the like. Owing to the multiplicity of their components a fusion of such substances is particularly easy to attain: but it is of importance, under what conditions such fusion is effected. The possibility of variation of the conditions in practice is offered by three variables, namely:

- (1.) Difference in temperature.
- (2.) Difference in the atmosphere of the furnace.
- (3.) Speed of melting down.

High temperature and oxidizing atmosphere yield slags of iron oxide of a high melting point. High temperature, reducing atmosphere and slow melting down yield metallic iron and slag of a high melting point. Rapid melting down in reducing atmosphere is capable of yielding particularly favourable working up conditions at lower furnace temperatures provided that conditions are observed, which are based on observations now to be stated:

Technical iron sulphide of about the eutectic composition  $\text{Fe}$ — $\text{FeS}$  has been fused in a furnace.

This melting down is carried out at a temperature of about 950°. The melt was then further heated and covered with coal until at temperature of about 1300°; roasted pyrites carrying zinc were 5 introduced into the melt covered still with coal. As soon as the added material has reached the furnace temperature, an intense reaction commenced, which is marked by the creation of heavy foam or froth. At the same time zinc vapours 10 escape, particularly if a temperature of from 1250° to 1350° is being maintained. By blowing air onto the bath the evolution of zinc may be accelerated. As melted products there is formed an iron-iron sulphide alloy of a higher specific weight and as 15 far as silicic acid be present as gangue an iron silicate slag of lesser specific weight, which separates out above the iron-iron sulphide layer.

The final aim of the process, as may be seen from the foregoing is to concentrate as far as possible the iron in the sulphide alloy and to keep the quantity of oxidic iron in the slag as low as possible. Now it has been found, that a considerable quantity of oxidic iron has passed into the iron-iron sulphide alloy as metallic iron; this was due 25 to the following reaction:



Oxidic iron may in this manner and by means of some sulphur only be completely converted into an iron-iron sulphide alloy. It must be the aim of the process to keep the quantity of iron, which in the presence of silicic acid is subject to scorification as low as possible. Now it has been ascertained that the deciding factor herein is the temperature, at which the iron oxide is melted down.

As an example the following mixture was fused:

|               | Grams |
|---------------|-------|
| 40 Iron oxide | 169   |
| Silicic acid  | 53    |
| Iron sulphide | 78    |

As long as a temperature of 1390° was not exceeded, this mixture yielded—130–160 gr. of slag, 120–100 gr. of iron-iron sulphide alloy with 10–14% sulphur. The slag contained 60–66% FeO, the balance being SiO<sub>2</sub>. If this fusion was however carried on at a temperature of more than 50. 1400°, a slag resulted with only 33% FeO, the balance being SiO<sub>2</sub>, whilst the iron-iron sulphide alloy showed a sulphur content of 7.8%. In order to establish that the composition of the melt was not accidental the process was repeated several 55 times and invariably the same result was obtained. The iron content in the slag was also independent of the sulphur content of the added iron sulphide, so that this scorification grade consisting of 33 percent by weight of FeO may be taken as an optimum of iron recovery for the range of temperature of from 1400°–1450°.

Having now in the preceding part described the basis of the new process and discussed the scientific principles of the same, I shall now proceed to a description of its technical carrying out.

Since both roasted pyrites as also crude pyrites or a mixture of both, are to be converted in a similar manner into Fe—FeS alloy, which is then to be worked up into metallic iron, it is a matter of course, that the preparatory steps for each of the materials are necessarily of a different character, whilst the furnace is always the same.

If it is necessary to work up roasted pyrites, which contain zinc or other volatile metallic compounds, the latter are placed after being

mixed with coal into a suitable smelting appliance. The following reactions take place:



They are accompanied by foaming and yield an iron-iron sulphide alloy, the further treatment of which will be described forthwith.

If it is a question of working up crude pyrites an addition of coal may not be necessary or may be so far reduced as to merely serve to protect the smelting bath from an excess of oxidation by the furnace gases. Whilst however when working roasted pyrites, provided the same have not been too insufficiently roasted, the sulphur content of the resulting iron-iron sulphide melt will remain relatively small, this content will increase considerably by melting down crude pyrites. In such a case therefore a reduction of the sulphur content of the iron-iron sulphide melt must be brought about by blowing air onto its surface, which sufficiently penetrates into the bath, to produce an oxidizing action. This oxidation of the sulphur by air does not however amount to a Bessemer process, as it is known for the treatment of copper matte or similar products. It has previously been stated, that in every phase of the known Bessemer process both sulphur and iron are oxidized and that after the termination of the process the whole of the iron is obtained in an oxidic slag. Also by prematurely interrupting such a copper-matte bessemering process a quantity of oxidized iron, accurately corresponding to the quantity of oxidized sulphur 95 is invariably obtained. The essential aim of this invention however is to avoid any oxidation of the iron almost completely and only to bring about that of the sulphur and even that only thus far, 100 until an iron-iron sulphide alloy with only 115 8–12% of sulphur has been formed. This may be attained by blowing air onto the surface. The experiments previously described have proved this to be possible. Although it had to be stated that in consequence of the presence of silicic acid 120 as gangue the formation of slag could not be completely avoided, it was on the other hand possible to show, that by keeping up a temperature of over 1400° the FeO content of same could be reduced down to about 33%. The quantity of 125 iron the oxidation of which into FeO is unavoidable, thus depends upon the quantity of the silicic acid (50% of the quantity of SiO<sub>2</sub>) and is therefore not too considerable as against the total quantity of iron to be treated. This also shows 130 the difference with the copper-Bessemer process, where, as is well known, silicic acid is separately added so as to convert and scoria all the iron into oxidic form. The bulk of the iron is secured by this new process as iron-iron sulphide alloy, 135 the sulphur content of which has now to be brought to such a grade, that the chilled alloy, i. e. granulated or cast into pigs or otherwise moulded, still retains a non-metallic character that is it may be disintegrated. Although this 140 process cannot yield the same volume of heat as a Bessemer process, leading to complete oxidation of the iron, there is a considerable amount of heat generated by the combustion of the sulphur, which, increased by that heat which is generated by the combustion of the coal on the surface of the bath, offers to a certain extent a compensation for the lack of iron combustion.

In working roasted pyrites this process naturally follows a more endothermic course, which 150

however may be appreciably compensated for by the addition of pyrites and thus effect a saving in heating energy. Inasmuch as zinc and other volatile metals cannot remain in a bath which is rich in metallic iron and poor in FeS, they are volatilized and can be separated from the gases discharged from the furnace. The slag is removed from the bath, the iron-iron sulphide melt granulated or made to quickly solidify in suitable forms. The granulated particles are converted by passing the same through a sintering apparatus into a sintered product of iron oxides, which have the value of natural magnetite free from gangue.

15 Further experiments have been made to provide means for the direct production of iron from an iron-iron sulphide alloy. A way was found to volatilize by known methods and by the addition of silicon the sulphur content of the iron-iron sulphide alloy in the shape of silicon sulphide. The possibility of doing so has not only been established, but also that the process occurred under a considerable development of heat. As the addition of silicon must exactly correspond with the sulphur content it is of course essential for economical grounds to carry the treatment of the ore so far as to lower the sulphur content of the iron-iron sulphide produced as far as ever possible, which is possible 30 within a limit of practically 4-6% of sulphur in the alloy.

Any metallurgic furnace could be used for carrying out the process. But since reverberatory furnaces, mainly used for the treatment of ores or metallurgical products with smelting baths, show a bad distribution of temperature insofar as uniform heating of the smelting bath is rendered difficult in consequence of bad thermal conduction the present process will be particularly effective if carried on in a furnace revolvable through 360° and in which the heating of the melting bath takes place both from the top and below. Such furnace is shown in Fig. 1 of the annexed drawing.

45 The charge H consisting for instance a mixture of roasted and unroasted pyrites in a proportion of 17:8, silicic acid and coal are introduced at E into the drum A and forms after being molten a bath B.

50 The heating gases are introduced at C in the direction of the arrows; passing through the furnace they leave the same at E and flow into the flue D.

E is a discharge-opening. The bath is covered 55 by a layer of coal G. The temperature is kept at about 1200° C.

If the process is carried on discontinually, a furnace of the short drum-type may be advantageously used, its diameter being about the same 60 as its length.

Such furnace is shown in Fig. 2 of the annexed drawing.

The charge is introduced at E into the drum A and forms after being molten a bath B. The 65 heating gases enter at C, H and leave the furnace at D. F is a discharging opening.

With furnaces of very great capacity, f. i. over 50 tons it will be advisable, to increase only the length of the furnace and corresponding to this lengthening of the furnace not to allow a return of the flames inside of the furnace but to pass them through the furnace to the end opposite to its entry. Lengthening of the furnace

permits to work particularly roasted pyrites by a continuous process. The roasted pyrites, with a suitable addition of coal are charged at the front side of entry of the flames and in view of the rapid liquefaction of the same in the bath it is possible to so operate the furnace that at the same time the corresponding quantity of iron-iron sulphide alloy continually leaves the furnace at the other end. The furnace itself has to maintain its continuous rotation since it is only possible in this way to keep up the even temperature of the melt.

What I claim is:

1. A process for the recovery of iron from iron and sulphur carrying metallurgical products, especially ores, consisting in melting the same with coal at a temperature of between about 985° C. and 1390° C. to form a molten iron-iron sulphide alloy with about 8% sulphur, separating the alloy and the slag, chilling, disintegrating and converting the alloy on a sintering apparatus into an agglomerate and recovering the iron therefrom in any appropriate manner.

2. A process for the recovery of iron from sulphur carrying metallurgical products, especially ores, consisting in melting the same with coal at a temperature of between about 985° C. and 1390° C. to form a molten iron-iron sulphide alloy containing about 8% sulphur, separating slag and alloy granulating and converting the alloy on a sintering apparatus into an agglomerate and recovering the iron therefrom in any appropriate manner.

3. A process for the recovery of iron from iron and sulphur carrying metallurgical products, especially ores, consisting in melting the same with coal at a temperature of between about 985° C. and 1390° C. to form an iron-iron sulphide alloy containing about 8% sulphur and introducing air into the charge, which is covered by a layer of coal, separating slag and the alloy, chilling, disintegrating and converting the same on a sintering apparatus into an agglomerate and recovering the iron therefrom in any appropriate manner.

4. A process for the recovery of iron and sulphur carrying metallurgical products, especially ores, consisting in melting the same with coal in a drum-furnace revolving through 360° at a temperature of between about 985° C. and 1390° C. to form a molten iron-iron sulphide alloy containing about 8% sulphur, the fresh charge being continuously introduced in the molten bath of the iron-iron sulphide alloy, separating the alloy from the slag, chilling, disintegrating and converting the alloy on a sintering apparatus into an agglomerate and recovering the iron therefrom in any appropriate manner.

5. A process for the recovery of iron from iron and sulphur carrying metallurgical products, especially ores, consisting in melting the same with coal in a drum-furnace of a short type, the diameter being about the same as its length, at a temperature of between about 985° C. and 1390° C. to form a molten iron-iron sulphide alloy, containing about 8% sulphur, the fresh charge being discontinually led into the furnace, separating the slag and the alloy, chilling, disintegrating and converting the same on a sintering apparatus into an agglomerate and recovering the iron therefrom in any appropriate manner.

ERNST JUSTUS KOHLMAYER.